

# United States Patent

[11] 3,619,167

[72] Inventor **Gordon James Marrs**  
**Bracknell, England**  
[21] Appl. No. **762,350**  
[22] Filed **Sept. 16, 1968**  
[45] Patented **Nov. 9, 1971**  
[73] Assignee **Imperial Chemical Industries Limited**  
**London, England**  
[32] Priority **Sept. 27, 1967**  
[33] **Great Britain**  
[31] **43,928/67**

[54] **HERBICIDAL COMPOSITIONS CONTAINING  
BIPYRIDYLUM SALTS WITH REDUCED  
CORROSIVENESS TOWARD METALS**  
6 Claims, No Drawings

[52] U.S. Cl. .... **71/94,**  
[51] Int. Cl. .... **252/395**  
[50] Field of Search. .... **A01n 9/22**  
71/87, 94;  
252/395; 260/296 Y, 925, 963

[56] **References Cited**  
UNITED STATES PATENTS  
2,734,869 2/1956 Mullen, Jr. et al. .... **252/395**

|           |         |                       |         |
|-----------|---------|-----------------------|---------|
| 2,841,486 | 7/1958  | Osborn et al. ....    | 71/87   |
| 2,989,392 | 6/1961  | Baker. ....           | 71/87   |
| 3,004,996 | 10/1961 | Arakelian et al. .... | 252/395 |
| 3,156,551 | 11/1964 | Brian. ....           | 71/94   |
| 3,228,960 | 1/1966  | Rigterink. ....       | 71/87   |
| 3,238,248 | 3/1966  | Rauhut. ....          | 71/87   |
| 3,340,041 | 9/1967  | Homer et al. ....     | 71/94   |
| 3,332,959 | 7/1967  | Braunholtz. ....      | 71/74   |
| 3,347,790 | 10/1967 | Meinhardt. ....       | 260/963 |
| 3,361,668 | 1/1968  | Wiese. ....           | 260/963 |
| 3,396,183 | 8/1968  | Brasch. ....          | 260/963 |

## OTHER REFERENCES

State Sci.-Res. etc; "Protecting Ferrous & Nonferrous Metals etc.," (1965) CA64 p. 410 (1966)

Teubel et al., "Basic Heavy-duty Lubricant for Diesel Engines," (1965) CA 65 p. 3650 (1966)

Primary Examiner—Lewis Gotts

Assistant Examiner—G. Hollrah

Attorney—Cushman, Darby and Cushman

**ABSTRACT:** Herbicidal compositions of bipyridylum diquaternary salts and a dithiophosphorous acid derivative. Examples of such derivatives are the salts of alkyl esters of dithiophosphoric acid.

HERBICIDAL COMPOSITIONS CONTAINING  
BIPYRIDIUM SALTS WITH REDUCED  
CORROSIVENESS TOWARD METALS

This invention relates to herbicidal compositions containing herbicidal bipyridium quaternary salts together with a corrosion inhibitor, and to a process for inhibiting the corrosion of metals by herbicidal bipyridium salts.

Herbicidal bipyridium quaternary salts have been disclosed in U.K. specifications 813,531 and 813,532. As disclosed in U.K. specifications 1,086,937, solutions of these compounds are somewhat corrosive toward metals. Aluminum metal and its alloys are particularly rapidly attacked. The chloride and bromide salts, which are preferred from the point of view of cost and of convenience in manufacture, are among the more corrosive salts formed from bipyridium quaternary cations. It has now been discovered that the corrosion of metals by solutions of bipyridium salts can be prevented or reduced by the incorporation of certain phosphorus acid derivatives into the solutions.

According to the present invention there is provided a herbicidal composition comprising a herbicidal bipyridium diquaternary salt and a phosphorus acid derivative of the formula



where  $R_1$  is an alkyl group of from one to 18 carbon atoms,  $R_2$  is an alkyl group of from one to four carbon atoms or an alkoxy group of from one to 18 carbon atoms, and  $M^+$  is a cation.

Examples of suitable cations include hydrogen ion ( $H^+$ ) alkali metal ion (for example,  $Na^+$ ), alkaline earth metal ion (for example  $\frac{1}{2}Mg^{++}$ ), and ammonium ion of the formula ( $N R_3 R_4 R_5 R_6$ ) $^+$  in which  $R_3$ ,  $R_4$ ,  $R_5$  and  $R_6$  each represent a hydrogen atom or an alkyl group (e.g. of 1-4 carbon atoms).

Examples of herbicidal bipyridium salts include the following:

1,1'-ethylene-2,2'-bipyridium dibromide (diquat dibromide)  
1,1'-dimethyl-4,4'-bipyridium dichloride (paraquat dichloride)  
1,1'-bis-3,5-dimethylmorpholinocarbonylmethyl-4,4'-bipyridium dichloride (morfamquat dichloride)  
1,1'-di-2-hydroxyethyl-4,4'-bipyridium dichloride  
1-(2-hydroxyethyl)-1'-methyl-4,4'-bipyridium dichloride  
1,1'-di-carbamoylmethyl-4,4'-bipyridium dichloride  
1,1'-di-N-methylcarbamoylmethyl-4,4'-bipyridium dichloride  
1,1'-bis-N,N-dimethylcarbamoylmethyl-4,4'-bipyridium dichloride  
1,1'-bis-N,N-diethylcarbamoylmethyl-4,4'-bipyridium dichloride  
1,1'-diacytonyl-4,4'-bipyridium dichloride  
1,1'-diethoxycarbonylmethyl-4,4'-bipyridium dibromide  
1,1'-diallyl-4,4'-bipyridium dichloride

The names in brackets set against the first three compounds in the above list are alternative names for these compounds in which the systemic chemical name for the cationic part of the compound has been replaced by the accepted common name for this entity. The bipyridium salts listed above are all chlorides or bromides, in which form they are most commonly encountered, but a wide range of other salts is also possible, for example those having iodide, phosphate, sulfate nitrate, methylsulfate, thiocyanate, cyanate, borate, bromate, perchlorate, acetate, oxalate, citrate, benzoate, phenylacetate, or succinate anions. Any desired salt may be used, since the herbicidal activity of the bipyridium salts is inherent in the cation and is independent of the nature of the anion.

Preferred compositions according to the invention are those which contain a phosphorus acid derivative of the above formula in which  $R_1$  is an alkyl group and  $R_2$  is an alkoxy group, and in which the total number of carbon atoms in  $R_1$  and  $R_2$  together is from eight to 14 carbon atoms.

A particularly preferred composition is that which contains a phosphorus acid derivative of the above formula in which  $R_1$  is an amyl radical and  $R_2$  is an amyloxy radical.

Further preferred compositions are those which contain a phosphorus acid derivative of the above formula in which  $R_1$  is an alkyl group of from five to 12 carbon atoms and  $R_2$  is a methyl group.

Compositions according to the invention may be solid or liquid. Solid compositions may contain for example, an inorganic salt as a diluent. Although solid compositions may be dry and relatively noncorrosive when freshly prepared, it is nevertheless desirable to incorporate a corrosion inhibitor, since the compositions may absorb moisture on storage and in any case are usually diluted with water before use. Liquid

compositions may comprise, for example, a solution or dispersion of the bipyridium salt in water containing a surface-active agent. Preferred surface-active agents are those which are nonionic. These include the condensation products of p octyl

and p-nonylphenol with ethylene oxide, for example the condensation product of p-nonylphenol with from seven to eight molar proportions of ethylene oxide sold under the name LIS-SAPOL ("LISSAPOL" is a trade mark). Other examples of nonionic surface-active agents include the condensation

products of ethylene oxide with mixtures of primary amines derived from coconut oil or soyabean oil fatty acids, for example those sold under the name ETHOMEEN ("ETHOMEEN" is a trade mark). Still further examples of nonionic surface-active agents include the N-oxides of condensation products of

ethylene oxide with cocoamine, for example those sold under the name AROMOX C15 ("AROMOX" is a trade mark).

Conveniently, the amount of the phosphorus acid derivative used in the compositions of the invention is from 0.01 to 10 percent of the weight of bipyridium cation present.

Preferably, the phosphorus acid derivative is used in an amount of from 0.5 to 5 percent by weight of the bipyridium cation present in the composition.

In another aspect the invention provides a process of inhibiting the corrosion of metals coming into contact with herbicidal bipyridium quaternary salts, by mixing the herbicidal bipyridium quaternary salt with a phosphorus acid derivative of the above formula, in which  $R_1$  is an alkyl group of from one to 18 carbon atoms,  $R_2$  is an alkyl group of from one to four carbon atoms, or an alkoxy group of from one to 18 carbon atoms, and  $M^+$  is a cation.

Compositions according to the invention are obtained by mixing the herbicidal bipyridium salt with the phosphorus acid derivative, further components of the composition being either present initially or added later as desired. In the case of an aqueous composition the pH of the solution may be adjusted to near pH7 if desired, although the phosphorus acid derivatives prevent or reduce corrosion over a wide range of pH values.

The invention is illustrated by the following examples.

EXAMPLE 1

This example illustrates the effectiveness of salts of certain 0,0-dialkyl esters of dithiophosphoric acids in reducing corrosion of aluminum by a solution of paraquat dichloride.

Test solutions were made up, having the following compositions:

|                                                                                                                                                         |      |
|---------------------------------------------------------------------------------------------------------------------------------------------------------|------|
| Paraquat dichloride (calculated as cation)                                                                                                              | 10%  |
| Sodium acetate                                                                                                                                          | 1.5% |
| Sodium benzoate                                                                                                                                         | 1.5% |
| AROMOX C15 ("AROMOX" is a Trade Mark), a surface-active agent, comprising the N-oxide of cocoamine condensed with 5 molar proportions of ethylene oxide | 1%   |
| Inhibitor                                                                                                                                               | 0.5% |

Water\*  
(\*The water contained sufficient sodium hydroxide to bring the initial pH of the solution within the range 6.5 to 7.5.)

For comparison, a control solution was prepared of the same composition except that the inhibitor was omitted. For the test, strips of British Standard 2L72 alloy were used. This comprises a composite of an aluminum alloy coated on each side with aluminum metal to a thickness of 5 percent of the alloy center. The overall thickness of the composite sheet was approximately 0.028 inch, and the composition of the central alloy portion was as follows:

| Component | % by weight |
|-----------|-------------|
| Copper    | 4.4         |
| Magnesium | 0.7         |
| Silicon   | 0.7         |
| Manganese | 0.6         |
| Aluminum  | to 100%     |

Strips of the aluminum alloy were immersed in the test solutions for 24 hours. Corrosion was assessed by determining the loss in weight of the strips. The results are given in table I below.

TABLE I

| Inhibitor              | Weight loss of aluminum strip (mg./cm. <sup>2</sup> /day) |
|------------------------|-----------------------------------------------------------|
| None (control).        | 10.5                                                      |
| <chem>CH3O</chem>      | 2.5                                                       |
| <chem>C2H5O</chem>     | 1.3                                                       |
| <chem>C2H5O</chem>     | 0.3                                                       |
| <chem>(CH3)2CHO</chem> | 0.03                                                      |
| <chem>C12H25O</chem>   | 0.2                                                       |
| <chem>C5H11O</chem>    | 0.2                                                       |

## EXAMPLE 2

This example illustrates the degree of inhibition of corrosion obtained using various concentrations of corrosion inhibitor in a solution of paraquat chloride. The test solutions were made up as in example 1 except for the variation in the concentration of the corrosion inhibitor, and the corrosion test was carried out as in example 1. Results are given in table 2 below

TABLE 2

| Inhibitor               | Inhibitor concentration (percent) | Weight loss of aluminum strip (mg./cm. <sup>2</sup> /day) |
|-------------------------|-----------------------------------|-----------------------------------------------------------|
| None (control solution) |                                   | 10.5                                                      |
| <chem>CH3O</chem>       | 0.01                              | 0.4                                                       |
| <chem>C12H25O</chem>    |                                   |                                                           |
| Same as above<br>Do     | 0.1<br>0.5                        | 0.3<br>0.03                                               |
| <chem>C2H5O</chem>      | 0.01                              | 1.3                                                       |
| <chem>CH32CHO</chem>    |                                   |                                                           |
| Same as above<br>Do     | 0.1<br>0.5                        | 1.2<br>0.3                                                |
| Do                      | 1.5                               | 0.3                                                       |

4  
EXAMPLE 3

This example illustrates the effectiveness of salts of certain 0-alkyl monoesters of methylphosphonothiolothionic acid in reducing corrosion of aluminum by a solution of paraquat dichloride. The aluminum was in the form of strips of the alloy used in examples 1 and 2. Test solutions were prepared having the following compositions.

|    |                                            |         |
|----|--------------------------------------------|---------|
| 10 | Paraquat dichloride (calculated as cation) | 10%     |
|    | Sodium acetate                             | 1.5%    |
|    | Sodium benzoate                            | 1.5%    |
|    | Inhibitor                                  | 0.5%    |
|    | Water*                                     | to 100% |

\*The water contained sufficient sodium hydroxide to bring the initial pH of the

15 For comparison a control solution was prepared having the same composition except that the inhibitor was omitted. Corrosion was determined as in example 1. The results are given in table 3 below:

TABLE 3

| Inhibitor            | Weight loss, mg./cm. <sup>2</sup> /day |
|----------------------|----------------------------------------|
| None (control)       | 10.2                                   |
| <chem>C5H11O</chem>  | 1.3                                    |
| <chem>C8H17O</chem>  | 0.3                                    |
| <chem>C11H23O</chem> | 0.3                                    |

## EXAMPLE 4

This example illustrates the effectiveness of sodium diamyl-dithiophosphate.



50 in reducing corrosion of aluminum coated alloy sheets by paraquat dichloride solution over a range of pH values.

The aluminum alloy was the same as that used in example 1. Test solutions were prepared as follows

|                                            |      |
|--------------------------------------------|------|
| Paraquat dichloride (calculated as cation) | 10%  |
| Sodium acetate                             | 1.5% |
| Sodium benzoate                            | 1.5% |
| Sodium diamyl-dithiophosphate              | 0.5% |

60 Water (containing varying amounts of sodium hydroxide) to 100%

A series of solutions containing the above ingredients and ranging in pH from 3.5 to 9.5 in steps of 0.5 pH unit was prepared. Corrosion assessment was carried out as in example 1, and it was found that the weight loss of the aluminum alloy in these solutions was  $0.5 \pm 0.25$  milligrams/cm.<sup>2</sup>/day over the pH range 3.5 to 9.5.

## EXAMPLE 5

70 This example illustrates the effectiveness of sodium diamyl-dithiophosphate



in reducing corrosion of aluminum alloy by paraquat diacetate. A test solution was prepared as follows: 100%

|                                           |         |
|-------------------------------------------|---------|
| Paraquat diacetate (calculated as cation) | 10%     |
| Sodium acetate                            | 1.5%    |
| Sodium benzoate                           | 1.5%    |
| Sodium diamyldithiophosphate              | 0.5%    |
| Water                                     | to 100% |

A control solution was prepared having the same composition except that the inhibitor was omitted. The aluminum alloy used was the same as that in example 1. Corrosion was determined as in example 1. The weight loss of the aluminum alloy in the solution containing no inhibitor was 6.2 milligrams/cm.<sup>2</sup>/day, while the weight loss of the aluminum alloy in the solution containing sodium diamyldithiophosphate was 0.5 milligrams/cm.<sup>2</sup>/day.

#### EXAMPLE 6

This example illustrates the effectiveness of sodium diamyldithiophosphate



in reducing corrosion of aluminum by diquat dichloride solution. A test solution was prepared having the following composition:

|                                          |         |
|------------------------------------------|---------|
| Diquat dichloride (calculated as cation) | 10%     |
| Sodium acetate                           | 1.5%    |
| Sodium benzoate                          | 1.5%    |
| Sodium diamyldithiophosphate             | 0.5%    |
| Water                                    | to 100% |

A control solution was prepared having the same composition except that the inhibitor was omitted. The corrosion test was carried out as in example 1. The weight loss of the aluminum alloy in the solution containing no inhibitor was 55 milligrams/cm.<sup>2</sup>/day, while the weight loss of the aluminum alloy in the solution containing sodium diamyldithiophosphate was 8 milligrams/cm.<sup>2</sup>/day.

#### EXAMPLE 7

This example illustrates an aqueous composition, according to the invention, comprising a herbicidal bipyridylum salt and a phosphorus acid derivative.

| Component                                                 | Percentage by weight |
|-----------------------------------------------------------|----------------------|
| Paraquat dichloride (calculated as cation)                | 20                   |
| Sodium acetate                                            | 1.5                  |
| Sodium benzoate                                           | 1.5                  |
| AROMOX C15 (AROMOX is a Trade Mark)                       | 2                    |
| Sodium diamyldithiophosphate                              | 0.5                  |
| SILCOLAPSE antifoaming agent (SILCOLAPSE is a Trade Mark) | 0.05                 |
| Water                                                     | to 100               |

#### EXAMPLE 8

This example illustrates an aqueous composition according to the invention, comprising a herbicidal bipyridylum salt and a phosphorus acid derivative.

| Component                                                 | Percentage by weight |
|-----------------------------------------------------------|----------------------|
| Paraquat dichloride (calculated as cation)                | 20                   |
| Sodium acetate                                            | 1.5                  |
| Sodium benzoate                                           | 1.5                  |
| AROMOX C15 (AROMOX is a Trade Mark)                       | 2                    |
| Compound 3 of table 3                                     | 0.5                  |
| SILCOLAPSE antifoaming agent (SILCOLAPSE is a Trade Mark) | 0.05                 |
| Water                                                     | to 100               |

What is claimed is:

1. A herbicidal composition of reduced corrosiveness toward metals in the presence of moisture comprising a herbicidal bipyridylum diquaternary salt and a corrosion inhibiting amount of (1) a phosphorus ingredient which consists essentially of a phosphorus acid derivative of the formula



30 wherein R<sub>1</sub> is an alkyl group of from one to 18 carbon atoms, R<sub>2</sub> is selected from alkyl groups of from one to four carbon atoms or alkoxy groups of from one to 18 carbon atoms, and M<sup>+</sup> is a cation selected from the group consisting of hydrogen ion, alkali metal ion, alkaline earth metal ion, and ammonium ion of the formula (N R<sub>3</sub> R<sub>4</sub> R<sub>5</sub> R<sub>6</sub>)<sup>+</sup> in which R<sub>3</sub>, R<sub>4</sub>, R<sub>5</sub>, and R<sub>6</sub> are selected from hydrogen or alkyl groups of one to four carbon atoms (2) a minor amount of sodium acetate and sodium benzoate and an inert carrier therefor, said composition containing a herbicidally effective amount of said bipyridylum salt.

35 2. A herbicidal composition according to claim 1 in which the group R<sub>2</sub> of the phosphorus acid derivative is an alkoxy group and the total number of carbon atoms in R<sub>1</sub> and R<sub>2</sub> together is from eight to 14.

40 3. A herbicidal composition according to claim 1 in which the group R<sub>1</sub> of the phosphorus acid derivative is an amyl radical and the group R<sub>2</sub> is an amyloxy radical.

45 4. A herbicidal composition according to claim 1 in which the group R<sub>1</sub> of the phosphorus acid derivative is an alkyl group of from five to 12 carbon atoms inclusive, and R<sub>2</sub> a methyl group.

50 5. A herbicidal composition according to claim 1 in which the phosphorus acid derivative is present to the extent of from 0.01 to 15 percent by weight of the bipyridylum cation in the composition.

55 6. A herbicidal composition according to claim 1 in which the phosphorus acid derivative is present to the extent of from 0.5 to 5 percent by weight of the bipyridylum cation in the composition.

\* \* \* \* \*